

June 22, 1937.

J. D. MORGAN ET AL

2,084,819

ELECTRIC HOT PLATE

Filed July 17, 1936

*Fig. 2.*



*Fig. 1.*



INVENTORS  
JOHN D. MORGAN  
BY RUSSELL E. LOWE  
*Edmund G. Borden*  
ATTORNEY

## UNITED STATES PATENT OFFICE

2,084,819

## ELECTRIC HOT PLATE

John D. Morgan, South Orange, N. J., and Russell E. Lowe, New York, N. Y., assignors to Power Patents Company, Jersey City, N. J., a corporation of Maine

Application July 17, 1936, Serial No. 91,136

2 Claims. (Cl. 219--37)

This invention relates to an electric hot plate, and is more particularly concerned with electric heating units of the closed top type having refractory resistor-supporting members employed for heating cooking vessels and the like.

Electric hot plates of the closed top refractory resistor-supporting type have long been known. The primary object of the present invention is to provide a refractory resistor-supporting closed top hot plate which shall be economical to build and which shall at the same time be more efficient and possess a longer life than hot plates previously known.

A feature of the invention resides in the use of chromium-iron-aluminum alloy wire as the resistor element. Such chromium-iron-aluminum wire has been found to have a working life at high temperatures which is very much longer than that of previously known metal and alloy resistance wire under comparable conditions. It has been found, however, that this new chromium-iron-aluminum alloy wire rapidly deteriorates and its efficiency as an electric resistor wire drops, when it is embedded in refractories containing alumina and silica of the type commonly used in constructing refractory resistor-supporting closed top hot plates. This deterioration of the chrome-iron-aluminum wire in the presence of alumina and silica refractory is apparently the result of a reducing action of the wire on the oxide refractory at the high operating temperatures at which the hot plate is used.

Another feature of the invention consists in embedding the chrome-iron-aluminum wire in a refractory resistor-supporting member comprising a phosphoric acid bonded zircon ferro-silicon-aluminum hydrate refractory of the type described in our copending application S. N. 37,662 filed June 27, 1936 for "High temperature refractory". This feature of the invention is based on the discovery that a zircon ferro-silicon refractory of the type described in our aforementioned application does not chemically react with chrome-iron-aluminum wire at temperatures as high as 2000-2300° F. and can therefore be used as the refractory resistor-supporting member for such wire in constructing closed top hot plates which are very efficient and which have a life many times that of hot plates now on the market.

With the foregoing and other objects and features in view, the invention consists in the improved electric heater and process of making same as hereinafter described and more particularly defined by the accompanying claims.

In the following description reference will be made to the accompanying drawing in which

Fig. 1 is a plan view, with parts cut away, showing the top of an electric hot plate constructed in accordance with the present invention and illustrating the manner of disposing the resistor coil of wire on the porcelain plate base member of the heating unit; and

Fig. 2 is a view in vertical side section showing the relative disposition of the porcelain plate, the coil resistor filament, and the refractory work-supporting surface of the plate imbedding the resistor filament.

In the following description the electric hot plate forming the subject of the present invention will be described chiefly by the method of manufacture. As shown in the drawing, the base member of the hot plate unit consists of a thin porcelain plate 10 (not substantially greater than  $\frac{1}{4}$  inch maximum thickness), said plate 10 preferably having a raised peripheral rim portion 12 and an axial bore 14 bounded by a raised central rim 16. Two small vertical apertures 18 are provided in the bottom of plate 10 at adjacent radially and circumferentially spaced points near the rim 12 for the purpose of receiving the terminal clamps or other connecting links between the two ends of a metal resistor heating coil 20 and an outside source of current (not shown) for supplying electrical energy for operating the hot plate. The resistor 20 consists of a chrome-iron-aluminum alloy wire constructed of 30-40% chromium, 5-8% aluminum and iron, together with—in some cases—a small amount (up to 5%) of cobalt. The hot plate in the present invention is made up from a helical coil of the alloy wire which is laid out in two concentric spirals which will fit within the rims 12 and 16 of plate 10, and which coil is annealed to lay flat on the plate 10 with its two ends 22 either attached to terminal posts mounted in the apertures 18 or carried out through the apertures as shown in the drawing.

As previously explained, the refractory work-supporting member 24 of the hot plate illustrated consists of a special type of refractory having properties which do not adversely affect the chemical composition and electric conductivity of the chrome-iron-aluminum wire 20 when associated therewith in intimate electrically uninsulated and heat conducting relation. This refractory is prepared substantially as follows:

Native zircon (zirconium silicate) is milled so that most of the milled material will pass through a 300 mesh screen. Ferrosilicon (preferably 75%

5

10

15

20

25

30

35

40

45

50

55

or 85% silicon) is ground to pass through an 80 mesh screen and be retained on a 300 mesh screen. Forty to fifty parts by weight of the milled grain zircon is wetted with water to a creamy consistency, and 6 parts by weight of 85% orthophosphoric acid is added to the wetted zircon. This mixture is digested for a period of about 12 hours at a temperature of 175-200° F. The digested zircon-phosphoric acid mixture is then well stirred and further diluted with water to what might be termed a "creamy" consistency. One part by weight of dry aluminum hydrate is mixed with 60 parts by weight of the milled ferrosilicon and the dry-mixed ferrosilicon and aluminum hydrate is added to the creamy partially digested zircon-phosphoric acid mixture. The resulting mixture is thoroughly agitated for a brief period and is then allowed to digest for about 12 hours at a temperature of 175-200° F. The latter period of digesting may be continued until such time as the digested mixture has dried to a solid condition, but preferably the final drying operation is conducted under a strong vacuum (20 inches or more) and thoroughly evacuated until all signs of gas ebullition from the mixture have ceased. This solid mixture is then ground and milled to pass through an 80 mesh screen, and is wetted with water to rehydrate the mixture to a molding or pouring consistency (about the consistency of cream).

Because the bonding agent for the refractory member 24 is phosphoric acid, some of which may not have completely reacted in the operation of preparing the refractory which has just been described, the following method of forming the member 24 has been adopted. The plate 10 is first laid or mounted on a rubber base or cushion, and the fluid zircon ferrosilicon aluminum hydrate refractory is then fed to the top of the plate 10 from a rubber container through a rubber hose. The fluid refractory is poured in two stages, the first stage being to about the level or height 26 to which the wire 20 extends above the top surface of the plate 10 (i. e. to approximately the outside diameter of the helical coil into which the wire is formed before placing it on the plate). The layer of refractory poured in the first stage is allowed to air set for a few minutes and then a second layer of refractory is poured to a level with the top of the rims 12 and 16. The heater is then

allowed to set and air dry for several hours, after which it is placed in a bake oven where it is heated slowly over a period of about 1½ hours to a temperature of approximately 550° F. and then heated more rapidly to a temperature of about 1250° F., at which temperature it is kept for a period of approximately half an hour. 5

After baking the plate and cooling, a glaze of suitable color may be applied in well known manner as by spraying, and the glaze is then dried and set by gradual heating to a temperature above 10 its softening point, followed by gradual cooling.

It will be understood that while the invention is not limited to the exact compositions of chrome-iron-aluminum alloy resistor wire and 15 of embedding zircon-ferrosilicon-aluminum hydrate refractory which have been stated in the example given, the invention resides particularly in the combination of alloy resistor wire and embedding refractory of the general type described whereby the life of a hot plate at high temperatures can be many times increased, and accordingly variations of substantially over plus or minus 5% in the composition of the alloy wire and in the composition of the refractory should 20 25 not be made.

The invention having been thus described, what is claimed as new is:

1. An electric heater comprising a thin porcelain base plate of low heat conductivity, a metallic resistor consisting of chrome-iron-aluminum wire wound in a helical coil and disposed on top of the plate with ends connected to closely spaced terminal elements, and a refractory work-supporting plate of high heat conductivity 30 35 mounting and bonded to the porcelain plate and embedding the resistor, said plate consisting essentially of a mixture of milled grain zircon, ferrosilicon and a small amount (about 1%) of aluminum hydrate bonded with the reaction products of phosphoric acid therewith. 40

2. An electric heater as described in claim 1, in which the alloy wire contains 30-40% by weight of chromium and 5-8% aluminum, and in which the refractory supporting plate contains 45 40-50 parts by weight of zircon and 50-60 parts by weight of 75% ferrosilicon bonded with about 6 parts by weight of 85% ortho-phosphoric acid. 45

JOHN D. MORGAN.  
RUSSELL E. LOWE. 50